

March 14, 1933.

I. DOROGI ET AL

1,901,150

INFLATABLE FIGURE TOY

Filed June 15, 1931

FIG. 1



FIG. 2



FIG. 3



Ivan Dorogi  
Lajos Dorogi  
INVENTORS

BY *MacK & Blum*  
ATTORNEY

## UNITED STATES PATENT OFFICE

ISTVÁN DOROGI AND LAJOS DOROGI, OF BUDAPEST, HUNGARY, ASSIGNEES OF ONE-HALF  
TO DR. DOROGI & CO. RUBBER GOODS FACTORY LIMITED, OF BUDAPEST, HUNGARY

## INFLATABLE FIGURE TOY

Application filed June 15, 1931, Serial No. 544,692, and in Hungary February 9, 1931.

When rubber is touched, the sensation is cold and unpleasant, and this is one of the objections to rubber toys. This disadvantage has been overcome up to now by uniting rubber with textile material, either by finishing rubberized fabric or by applying a textile cover to the rubber article, the latter being more or less independent from the said cover. However, such textile cover substantially 5 prevented the rubber from stretching, which was a great disadvantage. It has already been proposed to provide varnished rubber toys with ornaments applied to the varnish. However such varnish greatly decreases the 10 stretch of the rubber.

This invention relates to an inflatable and deflatable hollow rubber article having thin walls, which is ornamented with fibres adhering thereto, said rubber surface being 15 provided wholly or only in parts thereof with a fibre cover consisting of individual loose fibres. Said cover permits the rubber to retain all or nearly all of its extensibility.

The invention is set forth in the following 20 description and drawing which illustrates preferred embodiments thereof.

In the drawing, Fig. 1 shows a side view 25 of an inflatable rubber toy in the non-inflated condition in the form of a cat obtained in known manner from four superposed rubber sheets by stamping and welding operation.

Fig. 2 is a cross section according to line A—A through the above toy in the inflated condition.

Fig. 3 is a portion of the rubber wall of 30 the toy in an increased scale. In this figure No. 1 is the rubber sheet forming the article; No. 2 the adhesive layer into which the fibres No. 3 are embedded with part of their length No. 4.

According to the invention such articles 35 are produced by applying to and pressing on the sticky rubber surface to be provided with the fibre cover, loose individual fibres so that parts of the fibres become more or less

imbedded in the rubber surface. Owing to the fact that these parts of the fibres cannot become felted but on the contrary are separated from each other by thin rubber films located between them,—and that on the other hand the unattached free ends of the fibres are individually movable without any substantial resistance,—the original extensibility of the rubber covered by the fibres remains practically unaltered. At the same time, 50 when the rubber layer is stretched or bent the individual covering fibres are not restrained by the adjoining fibres, so that they can follow the movements of the rubber layer and then return to their original position, so that their attachment is substantially unaffected by such use.

By the use of individual and separated fibres it became for the first time possible to 55 produce inflatable rubber toys f. i. animal figures which are extensible so that they can be easily inflated and shaped and which have a completely new and artistic appearance and warm surface feel.

The attachment of the fibres can be accomplished in many ways. Some examples of 60 carrying out the invention are described hereafter.

In the simplest way, the attachment of the fibres is effected by swelling the raw rubber surface by treating it with a solvent or a swelling agent, so that this surface becomes similar to a sticky layer of rubber solution. After removal of the excess solvent but prior 65 to the complete drying of the sticky layer this surface is strewn with fibres of f. i. 2-3 mm. length of any desired origin. After strewing, it is advisable to exert on the surface now covered with fibres a moderate pressure (f. i. 70 by means of a rubber air cushion), whereby the entry of the fibres into the adhesive layer is promoted. After complete drying vulcanization is effected in the usual manner.

However, if the articles have very thin 75 walls it might happen that owing to the ac-

tion of the swelling agent the inner layers of the walls also may soften and may be distorted during the subsequent operations. Again sometimes rubber has a composition 5 which when swelling does not give a sufficiently sticky surface. In such cases it is possible to effect the swelling of the rubber by means of a swelling agent containing an adhesive. However it is more advisable to 10 accomplish the attachment of the fibres by means of a separate adhesive layer.

Accordingly an inflatable and previously vulcanized animal figure, assembled from sheets of about 0.3-0.4 mm. thickness, is coated by dipping with a rubber benzol solution 15 of 10-20% concentration mixed with 0.5-1 of a sticky resin soluble in benzol, such as mastic or the like. After draining off the solution the fibre-cover is applied according to the 20 preceding example. Subsequent to drying, the article is vulcanized in the vapor of sulphur chloride. Preferably the vulcanization is effected by heat, in which case the rubber solution naturally must contain, in addition 25 to the above mentioned basic materials, the material necessary for the hot vulcanization, such as sulphur, accelerator, fillers etc. In some cases it is possible to coat the article in a still unvulcanized condition with the rubber 30 solution and thereafter with the fibre cover, whereby one vulcanizing operation can be dispensed with.

When dipping articles of complicated shape 35 into the rubber solution mixed with the adhesive, and in the draining-off operation, it is often inevitable that due to the flowing off of the rubber solution too much rubber solution remains at some places and too little of the rubber solution remains adhering at other 40 places. In order to avoid this disadvantage it is possible to proceed so that the vulcanized or unvulcanized article to be coated with the fibre-cover is first dried perfectly or nearly perfectly after dipping it into the rubber 45 solution mixed with the adhesive, and to swell it thereafter again by dipping the adhesive layer into benzol, and to then first apply fibres. The advantage of this method of working consists in that during immersion in 50 the solvent a uniform thickness of the dried rubber layer swells throughout, so that the whole article will be coated with a uniform adhering layer. Instead of dipping, the rubber solution can be applied to the article in 55 any other known manner. If it is desired not to coat the whole article but only a part or parts of its surface with the fibre-cover, then either the surface will be coated with the rubber solution only at said part or parts and 60 strewn with the fibres. If desired, larger parts might be coated with the rubber solution but when the fibres are spread, said part or parts should be protected by a superposed stencil or the like. If necessary, the fibre- 65 cover can be partly or wholly dyed before or

after vulcanization prior or subsequent to applying it to the article. The improved article has a surface which is of fabric-like appearance, and the improved article can be repeatedly stretched and otherwise handled, 70 without losing this characteristic surface appearance.

The fibres can be of any desired origin, but the fibrous waste of the textile industry is preferably used. According to quality various effects can be attained. Thus very short cotton fibres yield an appearance and grip 75 very similar to buck skin or flannel. On the other hand skins can be imitated by using long fibres. Rubber toys which are thus made can 80 have their rubber walls stretched more than one hundred per cent.

We claim:

1. An inflatable and deflatable hollow rubber toy, having a rubber wall, said rubber wall being freely stretchable, the outer surface of said wall having separated fibres connected thereto so that the stretchability of said rubber wall is substantially undiminished. 85

2. A hollow rubber toy having a wall which is made of rubber, said rubber wall being freely stretchable, the outer surface of said wall having a film of rubber thereon, said film having separated fibres connected thereto, said fibres being sufficiently separated so that the stretchability of said rubber wall is substantially undiminished. 95

3. A hollow rubber toy, having a wall which is made of rubber, said rubber wall being freely stretchable, the outer surface of said wall having a film comprising rubber and an adhesive, said film having separated fibres connected thereto, said fibres being sufficiently separated so that the stretchability of said rubber wall is substantially undiminished. 100

4. A hollow rubber toy having a wall which is made of rubber, said rubber toy being freely stretchable, the outer surface of said wall having a film of rubber thereon, said film having separated fibres connected thereto, said fibres being sufficiently separated so that the stretchability of said rubber wall is substantially undiminished, said film of rubber being vulcanized. 110

5. A hollow rubber toy, having a wall which is made of rubber, said rubber wall being freely stretchable, the outer surface of said wall having a film comprising rubber and an adhesive, said film having separated fibres connected thereto, said fibres being sufficiently separated so that the stretchability of said rubber wall is substantially undiminished, said film of rubber being vulcanized. 120

6. An inflatable and deflatable hollow rubber toy having a rubber wall, said rubber wall being freely stretchable, the outer surface of said wall having separated fibres connected thereto so that said outer surface has a fabric- 125

like appearance, said fibres being sufficiently separated so that the stretchability of said rubber wall is substantially undiminished, so that said rubber wall can be stretched 5 without having its surface lose said fabric-like appearance.

In witness whereof we have signed hereunto our names.

10

ISTVÁN DOROGI.  
LAJOS DOROGI.

15

20

25

30

35

40

45

50

55

60

65